

Patented Feb. 23, 1932

1,847,015

# UNITED STATES PATENT OFFICE

JOHN F. McCAMBRIDGE, OF WASHINGTON, DISTRICT OF COLUMBIA

## CORROSION PREVENTING COMPOSITION

No Drawing. Application filed May 26, 1927, Serial No. 194,546. Renewed January 22, 1930.

This invention relates to compositions for preventing corrosion on metal surfaces and more particularly to such compositions for use in preventing after-corrosions in fire arms.

The corrosion of metal surfaces and particularly that known as after-corrosion in fire arms has been a serious problem and no satisfactory method or composition for eliminating such corrosion has been obtained to date, even though repeated efforts have been made with this end in view. See for example Technical Paper No. 188 of the Bureau of Mines. Many of the compositions which the prior art has suggested for these purposes fail utterly to accomplish the end sought. To a large extent the after-corrosion in fire arms appears to be due to the deposition of salts, such as potassium chloride, probably formed by decomposition of the potassium chlorate used in the powder or other explosive. The salt is deposited as the result of such decomposition and leads to corrosion, particularly in humid atmospheres.

Among the objects of the present invention are the production of a composition which is economical to manufacture but which will prevent the corrosion of such metal surfaces, and particularly the after-corrosion of fire arms.

Other objects and advantages will appear from the more detailed description set forth below, it being understood, however, that such more detailed description is given by way of illustration and not by way of limitation, since various changes may be made therein by those skilled in the art without departing from the scope and spirit of this invention.

Primarily it has been found that a phenol such as carbolic acid acts to eliminate the corrosive action on metal surfaces, and particularly that known as after-corrosion in fire arms. The phenol is desirably used with a base of oily character such base being an unctuous material such as vegetable, mineral and animal or fish oils, whether in the liquid or solid or semi-solid state. The base such as an oil is mixed with the phenol in any desired way, either at atmospheric temperatures or higher temperatures, the latter not being

necessary, but being desirable in some instances in order to get more rapid commixture. Agitation may be used if desired, but is not necessary.

It has been found that the ability of such compositions to prevent corrosion and particularly after-corrosion varies with the percentages of phenol present with the oil, such ability varying from non-effectiveness with zero per cent of phenol to complete effectiveness with definite percentages of phenol, depending upon the amount and nature of the salt or other corrosive element to be dissolved.

The compositions made in accordance with this invention are used in the following manner. The steel or other surface carrying the deposited salt or other corrosive agent is placed in contact with the composition and may be allowed to remain in such contact either indefinitely or until the next application of the salt is to be made on the steel surface. The oily material may or may not be removed at this time at the election of the user. It is undesirable to wipe off or otherwise remove the composition immediately after it has been applied, as more desirable results are obtained by prolonged contact between the metal surface and the composition. The maximum complete effectiveness is obtained when the solution is applied to all of the metal surface that has been exposed to the salt, and then left there to permit its action to ensue. This action takes place at ordinary atmospheric temperatures, and appears to be assisted rather than retarded by the presence of moisture. It should be noted

that after-corrosion of fire arms or corrosion of this character does not take place in the absence of moisture. If the steel or other metal surface to be treated is the bore of a fire arm, for example, the solution may be applied with a bristle brush of appropriate caliber. This method of application is more desirable than is the use of a cloth known as a "patch" for the reason that the bristle brush delivers the oil into the shoulder formed at the junction of the lands and grooves of a rifle fire arm, which result may not be obtained by the use of a "patch". When

the steel or other metal surface to be treated is to be stored for long periods, such, for example, as from two weeks to several years, it is desirable to use a base in the form of a grease, rather than a light oil, the latter being subject to evaporation.

As a general rule a treatment lasting for 24 hours is sufficient for complete absorption of the salts and the composition may be removed after this time without fear of corrosive action due to such salts, taking place.

The following examples will illustrate some of the specific compositions that may be used for these purposes.

## 15

## I

50 grains of phenol crystals are added to 1 ounce of sperm oil. The solution is readily obtained, particularly at approximately 150°

20 F. This composition may then be applied to steel or other metal surfaces. For example, in fire arms, it will serve to prevent the corrosion of the steel, due to the potassium chloride deposited on the steel under 25 heat and pressure, which potassium chloride may be derived from the potassium chlorate in the primer. The application of this solution to the steel surface upon which the salt has been deposited completely prevents corrosion by such salt. The oil in the composition also prevents oxidation or corrosion from ordinary causes.

## II

35 A further and preferred composition is made as follows:

30 grams of liquid phenol U. S. P. having a content of not less than 87 per cent pure phenol is mixed with 900 c. c. of lard oil.

40 Commixture is obtained readily without heat. This composition may be used in the manner set forth above.

Having thus set forth my invention, I claim:

45 1. A composition preventing corrosion on metal surfaces which consists of carbolic acid and lard oil in proportion sufficient to prevent after corrosion in firearms.

50 2. A composition preventing after corrosion in firearms which consists of 30 grams liquid phenol U. S. P. containing not less than 87 per cent pure phenol and 900 c. c. of lard oil.

55 3. The method of preventing after corrosion in fire arms which comprises applying thereto a composition containing phenol and lard oil.

In testimony whereof I hereunto affix my signature.

60 J. F. McCAMBRIDGE.